

# UNITED STATES PATENT OFFICE.

WILLIAM R. WALKER, OF NEW YORK, N. Y.

## MANUFACTURE OF STEEL.

1,155,849.

Specification of Letters Patent.

Patented Oct. 5, 1915.

No Drawing.

Application filed August 24, 1909. Serial No. 514,582.

*To all whom it may concern:*

Be it known that I, WILLIAM R. WALKER, of the city, county, and State of New York, have invented a new and useful Improvement in the Manufacture of Steel, of which the following is a specification.

My invention relates to the manufacture of steel by the use of the electric furnace succeeding the Bessemer converter or open hearth furnace; and is designed to reduce the expense of manufacture and make the steel more uniform and better in quality.

In the ordinary manufacture of steel the manganese contained in the pig iron is almost wholly lost through oxidation in the Bessemer converter or open hearth furnace. In such practice it is necessary to add manganese, or an alloy thereof, to obtain the desired quality of steel.

My invention is designed to wholly or largely avoid the addition of manganese to the steel; and to utilize the larger portion of the manganese contained in the pig iron. This manganese performs a very useful function in the electric furnace, owing to its effect on the oxidized iron of the bath. Heretofore, however, it has been considered necessary to reduce the manganese to a small proportion of the original amount, in the Bessemer or open hearth heat; and this manganese which is lost must be replaced by manganese additions.

I have found that when Bessemer converter or open hearth furnace is used in connection with an electric furnace I can obtain important advantages by stopping the heat short of the usual point, and at a stage where a large part, and preferably the major portion of the manganese is retained in the bath. I have also found that where a series of converters or open hearth furnaces is used, variations in the manganese content of the partly reduced heats may be equalized by supplying a mixer of large capacity between the converters or open hearth furnaces and the electric furnace. This mixer is adapted to hold a number of heats or charges at one time; and provides a constant and steady supply of metal to the electric furnace, while equalizing the percentage of metalloids in the metal taken to the electric furnaces. It is also of advantage in giving heats of more uniform duration and affording a more uniform product from the electric furnaces. In addition to this mixer between the steel mak-

ing apparatus and the electric furnaces, I also preferably provide an additional receiver or ladle on the casting side of the electric furnaces, and which is adapted to hold charges from a number of these furnaces at one time. From this receptacle, or large ladle, on the casting side of the electric furnaces, the metal may be tapped or poured into the ladles, by which it is taken to the molds. This additional receiver will aid in equalizing the variations in the product of the various electric furnaces, thus insuring a more uniform product. The mixer and the receiver may be heated either electrically or by gas, or any other desirable way.

In carrying out my process, therefore, I stop the heat of the Bessemer converter or open hearth furnace before it is carried to the usual point, and while a large and preferably a major percentage of the contained manganese is present in the metal, the manganese remaining being above .10 per cent. I then tap or pour these heats and feed them into the intermediate mixer. From this mixer, in which a dominant pool is preferably maintained, I take charges of a desirable size to the electric furnaces. The metal carried to the electric furnace will be equalized in manganese content and will carry a larger portion of the manganese that is now obtained. In the electric furnace the metal is deoxidized, largely through the action of manganese. I, therefore, wholly or largely avoid the addition of manganese to the electric furnace and utilize that contained in the original pig iron for this purpose. In my preferred practice I then tap or pour the charges from the electric furnace and feed them into the large ladle or receiver where the metal is further equalized, and from which it is tapped or poured into smaller ladles and poured into the molds.

The advantages of my invention result: 1st—from the retention of the manganese, or a large part of it in the heats from the converter or open hearth; 2nd—from the use of a mixer between the steel making apparatus and the electric furnaces. This mixer equalizes the large variations in manganese which would otherwise occur in the metal taken to the electric furnace, resulting from the inability to make the blows or heats of the same extent, or carry them to the same point in manganese extraction.

The converter is preferably acid lined;

and the open hearth may be either basic or acid; the electric furnace is preferably basic lined; but apparatus of various kinds may be used, and variations may be made in the 5 steps of my process, without departing from my invention.

I claim:

1. In the manufacture of steel, the steps comprising treating molten iron containing 10 a percentage of manganese in a Bessemer converter or open hearth furnace, stopping the treatment while the percentage of manganese is relatively high, transferring the heated metal to a basic-lined electric 15 furnace and treating it therein.
2. In the manufacture of steel, the steps comprising treating molten iron containing a percentage of manganese in a Bessemer converter or open hearth furnace to remove 20 at least a part of the silicon and carbon, then before the elimination of a considerable percentage of the manganese transferring the metal to a basic-lined electric furnace and treating it therein.
3. In the manufacture of steel, the steps comprising treating molten iron containing a percentage of manganese in an acid-lined 25 Bessemer converter or an open hearth furnace for the removal of at least a part of the silicon and carbon and retention of a portion of the manganese, and after the 30 elimination of the greater percentage of silicon and carbon and the removal of a less percentage of manganese, transferring the 35 metal to a basic-lined electric furnace and treating it therein.
4. In the manufacture of steel, the steps comprising treating molten iron containing a percentage of manganese, in a Bessemer 40 converter or open hearth furnace, until the manganese is reduced to not lower than .10 per cent., and then transferring the metal to a basic-lined electric furnace and treating it therein.
5. In the manufacture of steel, the steps comprising treating molten iron containing a percentage of manganese in an acid-lined 45 Bessemer converter or open hearth furnace

for the removal of at least a part of the silicon and carbon and retention of a portion of the manganese, and after the elimination of the greater percentage of silicon and carbon and the removal of a less percentage of manganese transferring the metal 50 to a mixer wherein the percentages of manganese are rendered more uniform, and thereafter transferring the metal to and treating it in a basic-lined electric furnace. 55

6. In the manufacture of steel, the steps comprising treating the molten iron containing a percentage of manganese in an acid-lined Bessemer converter or an open hearth furnace, transferring the metal before the completion of the heat to a metal mixer wherein the metals of uniform heats 60 are rendered uniform, then transferring the metal to and treating it in an electric furnace, and thereafter transferring it to a receiver whereby any variations in the content 65 of the charges from the electric furnace are 70 compensated for.

7. In the manufacture of steel, the steps comprising treating molten iron in a Bessemer converter or open hearth furnace, stopping the heat while the manganese percentage is relatively large, then treating the 75 resulting metal in a plurality of electric furnaces, and mixing the steel taken from the plurality of such electric furnaces.

8. In the manufacture of steel, the steps 80 comprising partially refining molten iron in a plurality of combustion furnaces, transferring the metal from said furnaces to a mixer, transferring successive charges of metal from the mixer to a series of electric 85 furnaces, purifying the metal in said electric furnaces, and then feeding the finished steel from said furnaces to a mixer and withdrawing the mixed metal from said mixer. 90

In testimony whereof, I have hereunto set my hand.

WILLIAM R. WALKER

Witnesses:

WILLIAM W. CORLETT,  
CLARENCE D. KERR.